

# United States Patent Office

2,738,327

Patented Mar. 13, 1956

1

2,738,327

## LITHIUM-STRONTIUM SOAP GREASES FROM OXIDIZED PETROLEUM FRACTIONS

George W. Eckert, Glenham, N. Y., assignor to The Texas Company, New York, N. Y., a corporation of Delaware

No Drawing. Application December 24, 1952,  
Serial No. 327,933

3 Claims. (Cl. 252—40)

This invention relates to improved lubricating grease 15 compositions and more particularly to lubricating greases containing mixed lithium and strontium soaps of oxidized petroleum fractions.

It is well known in the art to employ oxidized petroleum fractions as the saponifiable material in grease making, and greases have been prepared from such materials employing various metals as the metal component of the waxate soap. However, these oxidates are considerably different in many respects from the natural fats and fatty acids in their grease making properties, and difficulties have been encountered in producing greases of the desired properties from these materials. The chief difficulty, which has been found in a greater or less extent with all greases of this type of the prior art, is the tendency of these greases to harden, or "set up," in storage. This hardening is very objectionable from the standpoint of marketability, and also seriously impairs the service characteristics of the greases for many purposes.

In accordance with this invention, very superior lubricating greases, having both excellent lubricating properties and storage characteristics, are obtained by employing as the essential thickening agent a mixed lithium-strontium soap of a saponifiable material resulting from the oxidation of a petroleum fraction, the mixed lithium-strontium soap comprising substantial proportions of each metal soap. The soap may suitably comprise lithium and strontium oxide soaps in a proportion of about 1 to 4 to about 4 to 1 by weight, and preferably in a proportion of about 1 to 1 to about 4 to 1 by weight. This mixed base soap is employed in a suitable oleaginous vehicle in varying amounts to produce greases for various purposes ranging from semi-fluid to very stiff. Ordinarily, the soap content of the grease will be from about 10 to about 45 per cent by weight.

The oxidates employed in preparing the greases of this invention are oxidized petroleum fractions containing considerable proportions of saponifiable materials, or separated saponifiable fractions of such oxidized petroleum fractions such as have been employed heretofore in grease making. They are obtained by oxidizing a petroleum fraction such as a lubricating oil fraction, crude or refined wax, slack wax, or petrodatum at elevated temperatures, by means of an oxidizing agent such as air or oxygen, and in the presence or absence of a catalyst. Preferably, the oxidates employed for this purpose are highly oxidized materials having saponification numbers in the range from about 175 to about 450.

The mixed lithium-strontium soaps are prepared from the petroleum oxidates by any of the conventional methods employed for obtaining mixed base soaps, such as by coprecipitation or by mixing separately prepared lithium and strontium soaps. They are most conveniently prepared by the coprecipitation method, that is, by saponification of the oxidate with lithium and strontium hydroxides or other suitable compounds to produce directly a mixed soap of the desired ratio of lithium

2

and strontium soaps. An excess of lithium or strontium hydroxide, or of both lithium and strontium hydroxides, beyond the amounts required to react with all of the saponifiable matter is employed in the saponification. Preferably, an excess of lithium or strontium hydroxide is added sufficient to give a free alkalinity of about 0.01 per cent to about 10 per cent by weight of the finished grease. In addition to these special soaps, the greases of this invention may contain any of the usual additives such as, for example, oxidation and corrosion inhibitors, extreme pressure agents, oiliness agents and so forth, as well as small amounts of additional thickening agents such as polymeric materials and solid lubricants such as carbon black. These greases may also be mixed or blended with greases of other types if desired to produce greases of special properties.

The oleaginous vehicle employed in the grease may be any suitable oil of lubricating characteristics, which may be of mineral, vegetable, animal or synthetic origin, such as have been employed heretofore in lubricating greases. Suitable mineral oils include both distillate and residual fractions from paraffinic, naphthenic or mixed base crude, ranging from fairly low to fairly high viscosities, such as from about 50 to about 1500 seconds Saybolt Universal viscosity at 100° F. These oils may be obtained by any of the usual refining methods such as acid treating, solvent extraction, and so forth. For certain purposes, such as for example the production of low temperature greases, various synthetic oils may be employed with particular advantage. As examples of suitable oils of this type may be mentioned high molecular weight aliphatic ethers, such as normal hexyl ether, the alkyl esters of benzoic and phthalic acids, and the aliphatic dicarboxylic acid di-esters, such as di-2-ethyl hexyl sebacate, di-(secondary amyl) sebacate, di-2-ethyl hexyl azelate, di-isooctyl adipate, etc.

The grease preparation is suitably carried out by charging a quantity of oxidate together with lithium and strontium hydroxides in proportionate amounts to a conventional grease making kettle, where the mixture is maintained at elevated temperature below about 220° F. with stirring, air blowing or other mechanical agitation until the saponification is complete. The temperature is then increased to about 270° F. or higher and maintained at this increased temperature for a time sufficient to accomplish dehydration. The lubricating oil included in the grease is preferably added to the initial charge also, or only a small amount of the oil may be added to the initial charge and additional oil added during the saponification or after the dehydration to obtain a grease of the desired consistency. Other saponifiable materials such as the natural fats and oils commonly employed in grease making may also be added where it is desired to obtain a mixed grease.

Greases prepared from mixed lithium-strontium oxide soaps as described above have been found to have very different storage characteristics from the other petroleum oxide greases of the prior art, in addition to generally excellent lubricating characteristics equivalent to those obtainable with the very expensive highly refined natural fats and fatty acids. It is particularly surprising that oxide greases of excellent lubricating characteristics are obtained employing this combination of metals, since attempts to produce greases employing both lithium oxide soaps and strontium oxide soaps separately have given very unpromising results, the greases produced being gel-like and unsatisfactory in texture and softening to an objectionable degree upon working. For example, a grease comprising 20 per cent of lithium oxide soap in a naphthene base lubricating oil having a Saybolt Universal viscosity at 100° F. of about 300 seconds, had an unworked penetration (ASTM) at 77° F. after two days of

174 and a worked penetration of 274. A grease comprising 20 per cent of strontium oxide soap in a lubricating oil of the same type had an original unworked penetration of 217 and a worked penetration of 312, and in addition it had a very low dropping point of only 222° F. However, greases prepared according to this invention by employing both lithium and strontium oxide soaps in combination have been characterized by excellent texture, and have tended to harden slightly rather than to soften upon working. In addition, these greases very unexpectedly showed no hardening upon storage even for long periods of time.

The following example is given as illustrative of the greases of this invention.

#### EXAMPLE

A lubricating grease was prepared from the following materials:

|                                        | Grams |
|----------------------------------------|-------|
| Wax oxidate                            | 3,304 |
| Mineral lubricating oil                | 5,600 |
| LiOH (10%) (aqueous solution)          | 8,000 |
| Sr(OH) <sub>2</sub> ·8H <sub>2</sub> O | 900   |

The wax oxidate employed had a neutralization number of 250, a saponification number of 390 and contained 14.0 per cent of unsaponifiables. It was obtained by oxidizing a paraffin wax obtained from a pressed distillate of SAE 10 grade. The oxidation was carried out at a temperature of 270° F., a pressure of 65 p. s. i. g. and an air rate of 20 cubic feet per hour per pound of charge.

The mineral lubricating oil was a refined naphthene base distillate oil having a Saybolt Universal viscosity at 100° F. of about 300 seconds.

The grease preparation was carried out by charging the above materials in the amounts given above to a steam-heated grease kettle and heating for two hours at 200° F., with continuous stirring, until the saponification was substantially complete. The temperature was then increased to 300° F., and the mass held at this temperature for two hours to dehydrate, after which the temperature was allowed to fall and the grease finally drawn at 216° F. A smooth, buttery grease was obtained. The following table shows the storage characteristics of this grease (Grease No. 7 of the table) as compared with those of greases prepared from the same mineral oil and oxides of the same type, but containing different metals in place of lithium-strontium combination.

Table

#### STORAGE STABILITY OF OXIDATE GREASES

| Grease No.                             | 1    | 2     | 3    | 4     | 5     | 6    | 7     |
|----------------------------------------|------|-------|------|-------|-------|------|-------|
| <b>Composition, calculated:</b>        |      |       |      |       |       |      |       |
| Metals                                 | Na   | Na:Ba | K:Mg | Li:Mg | Na:Sr | K:Sr | Li:Sr |
| Ratio of metal soaps                   | 3:2  | 3:2   | 2:1  | 1:1   | 3:2   | 3:2  | 3:2   |
| Soap content, percent                  | 25.1 | 23.8  | 28.0 | 28.0  | 22.3  | 28.3 | 32.8  |
| Excess alkali, percent                 | 0.0  | 0.0   | 3.5  | 2.3   | 4.0   | 4.4  | 5.6   |
| Unsaponifiable (from oxidate), percent | 3.5  | 3.1   | 3.8  | 4.2   | 2.5   | 2.9  | 5.0   |
| Phenylalphanaphthylamine, percent      | 0.6  | 0.5   | 0.4  | 0.5   | 0.0   | 0.0  | 0.0   |
| Mineral oil, percent                   | 70.8 | 72.6  | 64.3 | 65.0  | 71.0  | 64.4 | 56.6  |
| <b>Penetration, ASTM, 77° F.:</b>      |      |       |      |       |       |      |       |
| Unworked basis:                        |      |       |      |       |       |      |       |
| Original grease                        | 285  | 324   | 343  | 222   | 289   | 336  | 357   |
| After 2 days                           | 227  | 201   | 217  | 157   | 198   | 185  | 365   |
| After 14 days                          |      | 182   |      | 154   |       |      | 376   |
| After 30 days                          | 180  | 164   | 167  | 150   | 183   | 113  | 365   |
| After 60 days                          |      | 140   |      |       |       |      | 360   |
| After 90 days                          |      |       |      |       |       |      | 362   |
| After 6 months                         |      |       |      |       |       |      | 1 379 |
| Worked basis:                          |      |       |      |       |       |      |       |
| Original grease                        | 298  | 331   | 316  | 245   | 287   | 271  | 338   |
| After 2 days                           | 291  | 310   | 201  | 263   | 307   | 264  | 342   |
| After 14 days                          |      | 312   |      | 253   |       |      | 342   |
| After 30 days                          | 288  | 319   | 279  | 261   | 309   | 235  | 348   |
| After 60 days                          |      | 283   |      |       |       |      | 346   |
| After 90 days                          |      |       |      |       |       |      | 340   |
| After 6 months                         |      |       |      |       |       |      | 1 349 |

<sup>1</sup> Sample containing 0.5% of PSF-34, a commercial amine-type oxidation inhibitor.

The above table shows the striking difference in storage characteristics between the lithium-strontium oxide grease and those of the other metal oxide greases representative of the oxidate greases of the prior art. As shown by the table, the lithium-strontium grease showed substantially no change in penetration on either the worked or the unworked basis during a six months' storage test. On the other hand, all of the other oxidate greases hardened continuously during storage on the basis of their unworked penetrations, with very large decreases in penetration occurring after only two days of storage. The lithium-strontium grease was also very resistant to change upon working, as shown by the small spread between the values found for the unworked and the worked penetrations during the test, and the change which occurred was a slight hardening instead of the softening which is a general characteristic of other oxidate greases in this test.

In addition to its excellent storage properties as discussed above, the lithium-strontium oxide grease of the example had all of the lubricating properties required of a very superior ball and roller bearing grease, as shown by the standard tests, including a dropping point of 407° F., a high mean Hertz load, without E. P. additives of 31, excellent water resistance, as shown by a loss of only 4 per cent in the dynamic water resistance test, and satisfactory rust resistance for an uninhibited grease. In addition, the Navy gear wear test (MIL-G-3278) on this grease was as follows: 0.4 gram weight loss, brass on steel, 5 pounds load, 1000 cycles; and 2.2 grams weight loss, brass on steel, 10 pounds load, 1000 cycles. These values are equivalent to those obtainable with good grade commercial ball and roller bearing greases. Very good results were also obtained with this grease in the torque breakdown machine test with a Federal ball bearing at 250° F., run continuously for 168 hours. The machine was shut down for observation at the end of this time with no failure. No grease leakage had occurred and the bearing condition was satisfactory.

Obviously, many modifications and variations of the invention, as hereinbefore set forth, may be made without departing from the spirit and scope thereof and, therefore, only such limitations should be imposed as are indicated in the appended claims.

I claim:

1. A lubricating grease comprising essentially an oleaginous vehicle as the chief constituent thickened to a grease consistency with a mixed lithium-strontium soap

of a saponifiable material obtained by the oxidation of a petroleum wax having a saponification number in the range from about 175 to about 450, said mixed lithium-strontium soap consisting of lithium and strontium soaps in a proportion by weight from about 1 to 4 to about 4 to 1, and containing free alkalinity in an amount equal to about 0.01 to about 10 per cent by weight of the grease,

2. Claim 1 wherein the soap consists of lithium and strontium soaps in about a 3 to 2 proportion by weight.

3. A lubricating grease comprising essentially a naphthene base distillate lubricating oil having a Saybolt Universal viscosity of about 100-400 seconds at 100° F. as the chief constituent, thickened with about 25-45 per cent by weight of a mixed lithium-strontium soap of a saponifiable material having a saponification number in the 15

range from about 350 to about 450, obtained by the oxidation of a petroleum wax, said mixed lithium-strontium soap consisting of lithium and strontium soaps in a proportion by weight of about 3 to 2, said lubricating grease containing about 4-10 per cent by weight of excess alkalinity.

References Cited in the file of this patent

UNITED STATES PATENTS

|           |          |               |
|-----------|----------|---------------|
| 2,409,950 | Meyer    | Oct. 22, 1946 |
| 2,417,428 | McLennan | Mar. 18, 1947 |
| 2,417,429 | McLennan | Mar. 18, 1947 |
| 2,669,543 | Hirsch   | Feb. 16, 1954 |